

Nov. 7, 1939.

T. V. GALASSI

2,179,289

TERRAZZO CONSTRUCTION

Original Filed May 21, 1935



Fig. 1



Fig. 2



Fig. 3



Fig. 4

*Inventor*  
Theodore V. Galassi

*By*  
Nathaniel Frucht

*Attorney*

## UNITED STATES PATENT OFFICE

2,179,289

## TERRAZZO CONSTRUCTION

Theodore V. Galassi, Providence, R. I.

Refiled for abandoned application Serial No. 22,508, May 21, 1935. This application February 13, 1939, Serial No. 256,181

8 Claims. (Cl. 94—3)

This application is a refiling of application Serial No. 22,508, filed May 21, 1935, and entitled Terrazzo construction.

My present invention relates to the building construction art, and has particular reference to the manufacture of terrazzo floors.

Terrazzo floors as at present built require a cement foundation or base, the terrazzo being spread over this base and provided with brass strips set therein at spaced intervals for the purpose of reducing setting shrinkage of the terrazzo and counteracting the effect of temperature expansion and contraction. The present practice utilizes brass strips approximately  $\frac{3}{16}$ " or more in width, and has disadvantageous features in that the brass strips are costly, and must be spaced relatively close together to properly take care of the expansive and contractive effect produced by temperature changes. I have found that the use of brass strips can be eliminated and shrinkage, expansion and contraction readily controlled by using a more suitable material, which lends itself to a greater variety of ornamental effects, and which permits the use of larger continuous areas of terrazzo than has heretofore been possible. It is the principal object of my invention to provide a better and more effective interlock material for terrazzo constructions.

Moreover, I have found it possible to change the terrazzo flooring so as to increase the attractive appearance thereof and at the same time improve its wearing qualities and durability. It is a further object of my invention to provide a novel terrazzo mixture which increases the life of the flooring and enhances its attractive appearance.

I have also found it advisable to provide a better and less costly base for the terrazzo, by utilizing materials which facilitate the formation of a proper foundation and at the same time decrease the weight thereof, whereby the dead weight of the completed floor is greatly decreased. It is a further object of my invention to provide a novel mixture of base materials having relatively light weight, which facilitate the formation of a suitable supporting base for the terrazzo layer.

The novel constructions above referred to have simplified the manufacture of terrazzo flooring, and the increased strength of the parts has permitted manufacture of complete prefabricated terrazzo units which may be readily transported to a building job for mounting, whereby complete units may be manufactured at low

factory cost, and may be quickly assembled on the job with a minimum of labor.

With the above and other objects and advantageous features in view, my invention consists of a novel arrangement of parts, and of novel compositions of material, more fully disclosed in the detailed description following, in conjunction with the accompanying drawing, and more specifically defined in the claims appended thereto.

In the drawing:

Fig. 1 is a plan view, broken away, showing an example of the appearance of a completed novel floor;

Fig. 2 is an enlarged section thereof on the line 2—2 of Fig. 1;

Fig. 3 is a perspective view of a prefabricated unit; and

Fig. 4 is an enlarged sectional detail thereof, showing the novel ingredients and their arrangement in the terrazzo layer and in the terrazzo base.

Referring to the drawing, the novel terrazzo flooring comprises terrazzo sections 10 which are separated by non-metallic strips 11, preferably of marble, and a foundation base 12, see Fig. 2, the marble strips 11 extending into the foundation base below the lower surface of the terrazzo layer. I have found that the use of marble strips, which have substantial width, compensate for the expansion and contraction of the terrazzo, whereby the sections may if desired be made as large as 25 to 50 square feet without danger of cracking, or separation because of temperature changes. I have also found that the use of marble strips permits a more pleasing and more attractive flooring, as the marble may be of any color and may be of different colors to suit the taste of the architect. The terrazzo layer, which normally consists of an aggregation or marble chip, a small percentage of carborundum particles and cement, is greatly improved both in appearance and in durability, by using a relatively large amount of fine carborundum aggregate. A terrazzo layer 10 one-half inch thick with marble chips 13 and a high percentage of carborundum aggregate 14, up to 40 per cent of the layer, with sufficient cement 15 for binding produces a very substantial solid layer of extremely great durability and wearing qualities, tests disclosing that it will wear twice as long as standard terrazzo flooring.

The usual terrazzo base is formed of sand and cement; this base is relatively heavy, and I have found it possible to simplify the manu-

10

25

30

35

40

45

50

55

facture of the base, lower the cost thereof, and greatly reduce the weight thereof, by utilizing sawdust as a substantial ingredient. Ordinary sawdust will not mix well; I have found it advisable to place the sawdust in water and soak it for an extended period of time, four days being suitable, after which the sawdust is removed and mixed with one part cement and one part coarse sand; the resultant mixture of sawdust 16, sand 17 and cement 18, see Fig. 2, is easily laid to provide a proper foundation which sets perfectly, and is much lighter in weight than standard foundations, whereby a completed floor consisting of a three-quarter inch base supporting a one-half inch terrazzo layer is one-third lighter than standard terrazzo flooring.

The improved base, which is lighter in weight and yet is very strong, and the terrazzo layer of great strength permits the manufacture of prefabricated units 19, such as illustrated in Fig. 3; blocks of flooring up to 25 square feet may be readily manufactured at the factory, and are strong enough to stand all handling during shipment and during laying without damage. The prefabrication permits setting under perfect conditions, as temperature, humidity, etc., are readily controlled, whereby all shrinkage when the blocks are laid is eliminated. I have thus found it possible to prefabricate flooring units, and to ship same to a construction job, where they are quickly laid upon a thin prepared foundation which preferably consists of a quarter inch layer of leveled cement. I have also found it feasible to prefabricate terrazzo strips, which can replace marble strips as above described, either for use at the construction job, or for the manufacture of the prefabricated block.

While I have described specific constructional embodiments of my invention, and specific compositions for the base and the terrazzo layer, it is obvious that changes in the arrangement of the parts and in the proportions of the ingredients used may be made to suit different architectural requirements, without departing from the spirit and scope of the invention as defined in the appended claims.

I claim:

1. In a terrazzo floor construction, a base consisting of a mixture of cement, sand and sawdust, spaced strips of marble embedded in said base and extending upwardly from the surface thereof, and terrazzo layers between said spaced strips. 5

2. A prefabricated building unit comprising a base consisting of a mixture of cement, sand and sawdust, spaced strips of marble embedded therein and extending from the surface thereof, and terrazzo layers between said strips. 10

3. A prefabricated building unit comprising a base, spaced strips embedded therein and extending from the surface thereof, and terrazzo layers containing from 20% to 40% fine carborundum 15 aggregate between said strips.

4. A prefabricated building unit comprising a base, spaced strips of material having a low coefficient of expansion embedded therein and extending from the surface thereof, and terrazzo 20 layers containing from 20% to 40% fine carbo-rundum aggregate between said strips.

5. A prefabricated building unit comprising a base, spaced strips of marble embedded therein and extending from the surface thereof, and terrazzo 25 layers containing from 20% to 40% fine carborundum aggregate between said strips.

6. A prefabricated building unit comprising a base consisting of a mixture of cement, sand and sawdust, spaced strips embedded therein and extending from the surface, and terrazzo layers containing from 20% to 40% fine carborundum aggregate between said strips. 30

7. A prefabricated building unit comprising a base consisting of a mixture of cement, sand and sawdust, spaced strips of material having a low coefficient of expansion embedded therein and extending from the surface thereof, and terrazzo 35 layers containing from 20% to 40% fine carborundum aggregate between said strips.

8. A prefabricated building unit comprising a base consisting of a mixture of cement, sand and sawdust, spaced strips of marble embedded therein and extending from the surface thereof, and terrazzo layers containing from 20% to 40% fine carborundum aggregate between said strips. 40 45

THEODORE V. GALASSI.